# EUROPEAN PATENT SPECIFICATION

(11) **EP 4 384 657 B1**
(45) Date of publication and mention of the grant of the patent: **08.10.2025**
(21) Application number: 22760941.9
(22) Date of filing: 03.08.2022
(51) Int. Cl.: C25C 5/02, C25C 1/12, C25C 1/20, C25C 7/08

(54) **PROCESS FOR ELECTROLYTIC PRODUCTION OF METAL POWDER**
VERFAHREN ZUR ELEKTROLYTISCHEN HERSTELLUNG VON METALLPULVER
PROCÉDÉ DE PRODUCTION ÉLECTROLYTIQUE DE POUDRE MÉTALLIQUE

(30) Priority: 13.08.2021 WO PCT/CN2021/112443
(43) Date of publication of application: 19.06.2024
(73) Proprietor: BASF SE, 67056 Ludwigshafen am Rhein (DE)
(72) Inventor: ZHU, Si Jun, Shanghai, Shanghai 200137 (CN); SONG, Jin Bo, Shanghai, Shanghai 200137 (CN); XIA, Jing Cheng, Shanghai, Shanghai 200137 (CN)
(74) Representative: BASF IP Association
(86) International application number: PCT/EP2022/071854
(87) International publication number: WO 2023/016896

(56) References cited:
- WO-A2-2015/095664
- CN-B- 106 629 738
- JP-A- 2003 342 775
- US-B1- 6 183 545

## Description

### FIELD OF THE INVENTION

The present invention relates to a process for electrolytic production of metal powder.

### BACKGROUND

Fine metal powders such as copper powder and silver powder are widely used in various applications, for example in electronic pastes, lubricants, catalysts, medicines and biofilters. Electrolytic deposition of metal powders has always been an important industrial process, as the process can provide metal powders with high quality under mild conditions and does not impose high requirements of starting materials.

US 6,183,545 describes an aqueous solution for the reductive deposition of metals comprising, besides water, (A) a special phosphine, and (B) a soluble compound of a metal or a compound of a metal solubilized through the formation of a soluble complex by said phosphine.

JP 2003-342775 relates to a method for producing silver powder, comprising the steps of: performing electrolysis using a silver plate as an anode in an acidic aqueous solution containing at least an alkyl group and a sulfo group and containing trivalent titanium ions; and generating silver powder by causing an oxidation-reduction reaction between the silver ions eluted from the silver plate and the trivalent titanium ions.

CN 106 629 738 describes a method for extracting silver from a crystalline silicon solar panel, comprising the following steps: dismantling solar cells from the crystalline silicon solar panel, removing an aluminum layer by using a sodium hydroxide solution, carrying out leaching with a mixed solution of organic acid and hydrogen peroxide so as to extract silver, electrolyzing the silver so as to obtain silver powder, and removing impurities with hydrofluoric acid so as to obtain a high-purity silicon material.

WO 2015/095664 relates to systems and methods for the recovery of noble metal from noble-metal-containing material, in which an electric current is transported between an electrode and the noble metal of a noble-metal-containing material to dissolve at least a portion of the noble metal from the noble-metal-containing material. The dissolved noble metal can subsequently be precipitated out of solution and recovered.

In conventional processes of producing copper powder by electrolytic deposition, an aqueous copper sulfate solution comprising sulfuric acid was generally adopted. The process needs certain measures for protection against corrosive sulfuric acid release from the electrolyte solution into ambient, particularly under an elevated process temperature. In conventional processes of producing silver powder by electrolytic deposition, an aqueous silver nitrate electrolyte solution comprising nitric acid was generally adopted. The process also has the problem of nitric acid release from the electrolyte solution into ambient under elevated process temperature.

Additionally, it was found by the inventors of the present invention that the deposition of silver particles on the cathode is accompanied with quick growth of dendritic aggregates, especially at the corner of the cathode, in the conventional processes using a silver nitrate electrolyte solution. The dendritic aggregates may extend to anode and thus increase the risk of short circuit.

There is still a need of alternative processes for producing copper powder and silver powder by electrolytic deposition. It is desirable that the processes can provide the metal powders having comparable or even improved quality than those obtained from those conventional processes.

### SUMMARY OF THE INVENTION

It is an object of the present invention to provide a process for production of copper powder and/or silver powder without using an electrolyte solution comprising any corrosive acid which may release into ambient under an elevated electrolysis temperature. A further object of the present invention is to provide a process for production of copper powder or silver powder with desirable or even smaller particle size.

It has been found that the objects of the present invention can be achieved by using an electrolyte solution comprising a metal sulfonate and a sulfonic acid.

Accordingly, in one aspect, the present invention provides a process for production of a powder of metal in an electrolytic cell comprising an anode made of the metal, a cathode and an electrolyte solution, which comprises
a) anodic dissolution to form ions of the metal in the electrolyte solution and cathodic deposition of metal particles from the electrolyte solution,
b) removal of the metal particles from the cathode into the electrolyte solution, and
c) isolation of the metal particles from the electrolyte solution,
wherein
- the metal is copper or silver, and
- the electrolyte solution comprises (i) an alkane sulfonic acid or alkanol sulfonic acid and (ii) a soluble metal salt of an alkane sulfonic acid or alkanol sulfonic acid.

The present specification also describes the copper or silver powder obtained or obtainable by the process as described herein.

The present specification also describes the use of an alkane sulfonic acid or alkanol sulfonic acid in an electrolyte solution for production of a silver or copper powder by electrolytic deposition.

### BRIEF DESCRIPTION OF THE DRAWINGS

Fig. 1 shows an SEM image of the copper powder as produced by the process according to the present invention, as described in Example 1.1.
Fig. 2 shows an SEM image of the copper powder as produced by a process not according to the present invention, as described in Comparative Example 1.1.
Fig. 3 shows an SEM image of the silver powder as produced by the process according to the present invention, as described in Example 2.1.
Fig. 4 shows a morphology picture of the silver deposit on the cathode as produced by the process according to the present invention, as described in Example 2.1.
Fig. 5 shows an SEM image of the silver powder as produced by a process not according to the present invention, as described in Comparative Example 2.1.
Fig. 6 shows a morphology picture of the silver deposit on the cathode as produced by a process not according to the present invention, as described in Comparative Example 2.1.
Fig. 7 shows particle size D₅₀ of the silver powder as produced by the process according to the present invention as described in Examples 2.1 to 2.3 and not according to the present invention as described in Comparative Examples 2.1 to 2.3.
Fig. 8 shows particle size D₉₀ of the silver powder as produced by the process according to the present invention as described in Examples 2.1 to 2.3 and not according to the present invention as described in Comparative Examples 2.1 to 2.3.

### DETAILED DESCRIPTION OF THE INVENTION

The present invention now will be described in detail hereinafter. It is to be understood that the present invention may be embodied in many different ways and shall not be construed as limited to the embodiments set forth herein. Unless mentioned otherwise, all technical and scientific terms used herein have the same meaning as commonly understood by one of ordinary skill in the art to which the present invention belongs.

As used herein, the singular forms "a", "an" and "the" include plural referents unless the context clearly dictates otherwise.

As used herein, the terms "comprise", "comprising", etc. are used interchangeably with "contain", "containing", etc. and are to be interpreted in a non-limiting, open manner. That is, e.g., further components or elements may be present. The expressions "consists of" or "consists essentially of" or cognates may be embraced within "comprises" or cognates.

As used herein, the term "aqueous" means that an electrolyte solution comprises a solvent containing at least 50% water. Preferably, at least 75%, more preferably 90% of the solvent is water. It can be contemplated that the solvent of the electrolyte solution consists essentially of water without any intentionally added organic solvent. Any type of water may be used, with preference to distilled or deionized water.

In the first aspect, the present invention provides a process for production of a powder of metal in an electrolytic cell comprising an anode made of the metal, a cathode and an electrolyte solution, which comprises
a) anodic dissolution to form ions of the metal in the electrolyte solution and cathodic deposition of metal particles from the electrolyte solution,
b) removal of the metal particles from the cathode into the electrolyte solution, and
c) isolation of the metal particles from the electrolyte solution,
wherein
- the metal is copper or silver, and
- the electrolyte solution comprises (i) an alkane sulfonic acid or alkanol sulfonic acid and (ii) a soluble metal salt of an alkane sulfonic acid or alkanol sulfonic acid.

As well-known, the anode is made of the metal to be deposited on cathode and thus supplies metal ions into the electrolyte solution continuously during the operation of the electrolytic cell. Generally, the anode may be made of the metal having a purity of at least 95%, for example at least 98% or at least 99%. In the process according to the present invention, the anode is made of copper or silver having a purity within above ranges.

There is no particular restriction to the material of cathode. The cathode useful for the process according to the present invention may be made of, for example, stainless steel or titanium.

The anode and the cathode may be arranged at a distance of 1 cm to 10 cm, preferably 3 cm to 6 cm, for example 3 cm to 5.5 cm.

The inventors of the present invention found that the electrolyte solution comprising (i) an alkane sulfonic acid or alkanol sulfonic acid and (ii) a soluble metal salt of an alkane sulfonic acid or alkanol sulfonic acid is effective for producing silver and copper powders under an elevated electrolysis temperature, without the problem of acid release into ambient.

Useful alkane sulfonic acids as the component (i) may be C₁-C₁₂-alkane sulfonic acids, preferably C₁-C₆-alkane sulfonic acids. The alkane sulfonic acids may be monosulfonic acids and disulfonic acids. Examples of alkane monosulfonic acids include, but are not limited to methanesulfonic acid, 1-ethanesulfonic acid, 1-propanesulfonic acid, 2-propanesulfonic acid, 1-butanesulfonic acid, 2-butanesulfonic acid, 1-pentanesulfonic acid, 1-hexanesulfonic acid, 1-decanesulfonic acid and 1-dodecanesulfonic acid. Examples of alkane disulfonic acids include, but are not limited to methanedisulfonic acid, 1,1-ethanedisulfonic acid, 1,2-ethanedisulfonic acid, 1,1-propanedisulfonic acid, 1,3-propanedisulfonic acid, 1,1-butanedisulfonic acid and 1,4-butanedisulfonic acid. One alkane sulfonic acid or any mixture of two or more alkane sulfonic acids may be used in the electrolyte solution in the process according to the invention.

Useful alkanol sulfonic acids as the component (i) may be C₂-C₁₂-alkanol sulfonic acids, preferably C₂-C₆-alkanol sulfonic acids, i.e., hydroxy substituted C₂-C₁₂-, preferably C₂-C₆-alkane sulfonic acids. The hydroxy may be on a terminal or internal carbon of alkyl chain of the alkane sulfonic acids. Examples of useful alkanol sulfonic acids include, but are not limited to 2-hydroxy-1-ethanesulfonic acid, 1-hydroxy-2-propanesulfonic acid, 2-hydroxy-1-propanesulfonic acid, 3-hydroxy-1-propanesulfonic acid, 2-hydroxy-1-butanesulfonic acid, 4-hydroxy-1-butanesulfonic acid, 4-hydroxy-2-butanesulfonic acid, 2-hydroxy-1-pentanesulfonic acid, 4-hydroxy-1-pentanesulfonic acid, 2-hydroxy-1-hexanesulfonic acid, 2-hydroxy-1-decanesulfonic acid and 2-hydroxy-1-dodecanesulfonic acid. One alkanol sulfonic acid or any mixture of two or more alkanol sulfonic acids may be used in the electrolyte solution in the process according to the invention.

The alkane sulfonic acids and alkanol sulfonic acids may be those prepared by any methods known in the art or commercially available ones without particular restrictions.

The alkane sulfonic acid or alkanol sulfonic acid as the component (i) may be comprised in the electrolyte solution at a concentration in a range of 1 to 200 grams per liter (g/L) of the electrolyte solution, particularly 5 to 180 g/L, preferably 10 to 150 g/L.

Herein, the soluble metal salt of an alkane sulfonic acid or alkanol sulfonic acid as the component (ii) refers to a soluble silver or copper salt of alkane sulfonic acid or alkanol sulfonic acid. The soluble silver or copper salt of alkane sulfonic acid or alkanol sulfonic acid will also be referred to as soluble metal sulfonate hereinbelow.

The alkane sulfonic acid or alkanol sulfonic acid from which the soluble metal sulfonate is derived may be same as or different from the alkane sulfonic acid or alkanol sulfonic acid as the component (i), and selected from those as described hereinabove for the component (i).

Preferably, the soluble metal sulfonate is a soluble silver or copper salt of the alkane sulfonic acid or alkanol sulfonic acid as the component (i).

For example, the electrolyte solution may comprise methanesulfonic acid as the component (i) and copper or silver methanesulfonate as the component (ii).

The soluble metal sulfonate as the component (ii) may be comprised in the electrolyte solution at a concentration in a range of 1 to 200 g/L of the electrolyte solution, particularly 5 to 150 g/L, preferably 5 to 120 g/L, calculated as the metal ions.

The electrolyte solution may be prepared by any known processes, for example by dissolving the metal (i.e., copper or silver), an oxide of the metal, a hydroxide of the metal, or a carbonate of the metal in a solution of the alkane sulfonic acid or alkanol sulfonic acid as described hereinabove, to provide a solution with desired concentrations of the metal ions and the sulfonic acid.

The electrolyte solution may optionally comprise one or more additives known useful in the art, for example, gelatins derived from collagen (e.g., animal glue), glucose, urea. Some inorganic additives may also be mentioned, for example cupric chloride to improve the electrical conductivity or adjust the pH of the electrolyte solution in the copper powder production. The additives, if present, may be comprised in the electrolyte solution at concentration of up to 20 g/L, more preferably up to 10 g/L.

In some embodiments, the present invention provides a process for production of silver powder in an electrolytic cell comprising an anode made of silver, a cathode and an electrolyte solution, wherein the electrolyte solution comprises (i) an alkane sulfonic acid or alkanol sulfonic acid and (ii) a soluble silver alkane sulfonate or alkanol sulfonate.

In those embodiments of the process for production of silver powder, the alkane sulfonic acid or alkanol sulfonic acid as the component (i) is preferably comprised in the electrolyte solution at a concentration in a range of 1 to 50 grams per liter (g/L) of the electrolyte solution, particularly 5 to 30 g/L, preferably 10 to 20 g/L. Additionally or alternatively, the soluble silver alkane sulfonate or alkanol sulfonate as the component (ii) is preferably comprised in the electrolyte solution at a concentration in a range of 50 to 200 g/L of the electrolyte solution, particularly 60 to 150 g/L, preferably 80 to 120 g/L, calculated as silver ions.

In some other embodiments, the present invention provides a process for production of copper powder in an electrolytic cell comprising an anode made of copper, a cathode and an electrolyte solution, wherein the electrolyte solution comprises (i) an alkane sulfonic acid or alkanol sulfonic acid and (ii) a soluble copper alkane sulfonate or alkanol sulfonate.

In those embodiments of the process for production of copper powder, the alkane sulfonic acid or alkanol sulfonic acid as the component (i) is preferably comprised in the electrolyte solution at a concentration in a range of 50 to 200 grams per liter (g/L) of the electrolyte solution, particularly 80 to 200 g/L, preferably 100 to 160 g/L. Additionally or alternatively, the soluble copper alkane sulfonate or alkanol sulfonate as the component (ii) is preferably comprised in the electrolyte solution at a concentration in a range of 1 to 50 g/L of the electrolyte solution, particularly 5 to 30 g/L, preferably 5 to 15 g/L, calculated as copper ions.

In step a), the anodic dissolution and cathodic deposition may be carried out at an ambient temperature or an elevated temperature, depending on the temperature of electrolyte solution.

For example, the process may be carried out at a temperature in the range of 20 °C to 70 °C, preferably 30 °C to 60 °C, more preferably 40 to 50 °C.

The electrolyte solution may be pumped at a flow rate of about 5 to 20 liters per minute (L/min) during step a). The electrolyte solution may be pumped from a reservoir into the electrolytic cell from the top and exit from the bottom of the electrolytic cell, or may be pumped into the electrolytic cell from the bottom and exit from the top of the electrolytic cell.

Step a) may be carried out at a current density in the range of 2 to 20 A/dm² (ASD), particularly 3 to 15 A/dm², for example 3 to 10 A/dm² for the production of silver powder, and 8 to 15 A/dm² for the production of copper powder.

The anodic dissolution and cathodic deposition in step a) are generally carried out for a period of 10 to 60 mins, for example 10 to 30 mins, before removing the metal particles deposited on the cathode in step b).

In step b), the metal particles may be removed from the cathode into the electrolyte solution by any mechanical means as well known in the art without any restriction.

In step c), the electrolyte solution comprising the metal particles as obtained from step b) are subjected to an isolation to provide the metal powder. Optionally, the isolated meal powder may further be subjected to a post treatment including washing, drying and/or anti-oxidation treatment. The post treatment may be carried out with any conventional means. For example, the isolated meal powder may be washed with deionized water, dried under vacuum and reduced under an atmosphere of hydrogen.

Accordingly, the process according to the present invention may further comprises following steps:
d) washing the metal particles isolated from step c), preferably with deionized water,
e) vacuum drying, and
f) anti-oxidation of the metal particles, preferably reduction under an atmosphere of hydrogen.

In some illustrative embodiments, the present invention provides a process for production of a silver powder in an electrolytic cell comprising an anode made of silver, a cathode and an electrolyte solution, which comprises
a) anodic dissolution to form silver ions in the electrolyte solution and cathodic deposition of silver particles from the electrolyte solution,
b) removal of the silver particles from the cathode into the electrolyte solution, and
c) isolation of the silver particles from the electrolyte solution,
wherein the electrolyte solution comprises (i) a C₁-C₆-alkane sulfonic acid or alkanol sulfonic acid and (ii) a soluble silver C₁-C₆-alkane sulfonate or C₁-C₆-alkanol sulfonate.

Preferably, in the illustrative embodiments of the process for production of silver powder, the electrolyte solution comprises (i) a C₁-C₆-alkane sulfonic acid or alkanol sulfonic acid at a concentration in a range of 1 to 50 g/L of the electrolyte solution, and (ii) a soluble silver C₁-C₆-alkane sulfonate or C₁-C₆-alkanol sulfonate at a concentration of 50 to 200 g/L of the electrolyte solution.

More preferably, in the illustrative embodiments of the process for production of silver powder, the electrolyte solution comprises (i) a C₁-C₆-alkane sulfonic acid or alkanol sulfonic acid at a concentration in a range of 5 to 30 g/L, preferably 10 to 20 g/L of the electrolyte solution, and (ii) a soluble silver C₁-C₆-alkane sulfonate or C₁-C₆-alkanol sulfonate at a concentration of 60 to 150 g/L of the electrolyte solution, calculated as silver ions.

Most preferably, in the illustrative embodiments of the process for production of silver powder, the electrolyte solution comprises (i) a C₁-C₆-alkane sulfonic acid or alkanol sulfonic acid at a concentration in a range of 5 to 30 g/L, preferably 10 to 20 g/L of the electrolyte solution, and (ii) a soluble silver C₁-C₆-alkane sulfonate or C₁-C₆-alkanol sulfonate at a concentration of 80 to 120 g/L of the electrolyte solution, calculated as silver ions.

In any of the illustrative embodiments of the process for production of silver powder, step a) is carried out at a temperature in the range of 40 to 50 °C, preferably 45 to 50°C.

In some other embodiments, the present invention provides a process for production of copper powder in an electrolytic cell comprising an anode made of copper, a cathode and an electrolyte solution, which comprises
a) anodic dissolution to form copper ions the in the electrolyte solution and cathodic deposition of copper particles from the electrolyte solution,
b) removal of the copper particles from the cathode into the electrolyte solution, and
c) isolation of the copper particles from the electrolyte solution,
wherein the electrolyte solution comprises (i) a C₁-C₆-alkane sulfonic acid or alkanol sulfonic acid and (ii) a soluble copper C₁-C₆-alkane sulfonate or C₁-C₆-alkanol sulfonate.

Preferably, in the illustrative embodiments of the process for production of copper powder, the electrolyte solution comprises (i) a C₁-C₆-alkane sulfonic acid or alkanol sulfonic acid at a concentration in a range of 50 to 200 g/L of the electrolyte solution, and (ii) a soluble silver C₁-C₆-alkane sulfonate or C₁-C₆-alkanol sulfonate at a concentration of 1 to 50 g/L of the electrolyte solution.

More preferably, in the illustrative embodiments of the process for production of copper powder, the electrolyte solution comprises (i) a C₁-C₆-alkane sulfonic acid or alkanol sulfonic acid at a concentration in a range of 80 to 200 g/L, preferably 100 to 160 g/L of the electrolyte solution, and (ii) a soluble silver C₁-C₆-alkane sulfonate or C₁-C₆-alkanol sulfonate at a concentration of 5 to 30 g/L of the electrolyte solution, calculated as copper ions.

Most preferably, in the illustrative embodiments of the process for production of copper powder, the electrolyte solution comprises (i) a C₁-C₆-alkane sulfonic acid or alkanol sulfonic acid at a concentration in a range of 80 to 200 g/L, preferably 100 to 160 g/L of the electrolyte solution, and (ii) a soluble silver C₁-C₆-alkane sulfonate or C₁-C₆-alkanol sulfonate at a concentration of 5 to 15 g/L of the electrolyte solution, calculated as copper ions.

In any of the illustrative embodiments of the process for production of copper powder, step a) is carried out at a temperature in the range of 40 to 50 °C.

The present specification also describes the copper or silver powder obtained or obtainable by the process according to the present invention as described herein.

The copper powder obtained or obtainable by the process according to the present invention has a particle size D₅₀ in the range of 20 to 120 microns (µm), preferably 30 to 100 µm, more preferably 40 to 90 µm, most preferably 40 to 80 µm.

The silver powder obtained or obtainable by the process according to the present invention has a particle size D₅₀ in the range of 100 to 600 microns (µm), preferably 150 to 500 µm, more preferably 200 to 400 µm. Alternatively or additionally, the silver powder obtained or obtainable by the process according to the present invention has a particle size D₉₀ in the range of 200 to 1,000 microns (µm), preferably 400 to 800 µm.

D₅₀ is the diameter value at which 50 % of the total number of particles as characterized consists of particles with a diameter less than the value, as measured by a particle size laser analyzer.

D₉₀ is the diameter at which 90% of the total number of particles as characterized consists of particles with a diameter less than this value, as measured by a particle size laser analyzer.

The present specification also describes the use of an alkane sulfonic acid or alkanol sulfonic acid in an electrolyte solution for production of a silver or copper powder by electrolytic deposition.

### Examples

### Description of Measurements in Examples:

Scanning electron microscopy (SEM): Zeiss Supra^{®} 55 from Carl Zeiss AG.

Particle size measurement: Malvern Mastersizer 2000G.

In each example, the current efficiency (η) was calculated in accordance with the following equation: $η = \frac{m}{q \times l \times t} \times 100 %$ in which
η represents current efficiency, expressed in %;
m represents mass of the metal powder deposited per cell over a period of t, expressed in g;
I represents electric current intensity, expressed in A;
t represents period of electroplating, expressed in hour; and
q represents electrochemical equivalent of the metal, which is 1.186 g/(A·h) for copper and 4.025 g/(A·h) for silver.

Electrical energy consumption (W) was calculated in accordance with the following equation: $W = \frac{U \times 1000}{η \times q} \times 100 %$ in which
W represents energy consumption, expressed in kW·h/t;
η represents current efficiency, expressed in %; and
U represents average bath voltage, expressed in V.

### Example 1 Production of Copper powder

### Example 1.1

Black CuO was dissolved in an aqueous diluent solution of methanesulfonic acid (MSA) to provide a solution containing 12 g/L of copper ions and 140 g/L of free methanesulfonic acid as the electrolyte solution. The solution was poured into an electrolytic cell and kept at a temperature of 40 °C. An anode of phosphorus copper plate and a cathode of titanium plate were arranged in the electrolytic cell at a distance of 5 cm. The electrolytic deposition was conducted by applying a direct current with the current density of 13 A/dm² for 15mins. Then, the obtained copper particles were removed from the cathode and isolated from the electrolyte solution. The collected copper particles were filtered with vacuum filtration and washed by DI water, dried at a temperature of 60 °C in a vacuum drying oven, then subjected to reduction treatment by heating to 500 °C in a reducing atmosphere of hydrogen.

The bath voltage is 2.3V, as determined by *Kocour* power supply, the current efficiency (η) is 89.32% and the electrical energy consumption (W) is 2171 kW·h/t. Sparse and thin dendritic crystals were observed via SEM for the copper powder, as shown in Figure 1. The copper powder has a particle size D₅₀ of 79.5 µm.

### Example 1.2

The process was carried out in the same manner as described in Example 1.1 expect that the electrolyte solution was kept at a temperature of 25 °C.

The bath voltage is 2.8 V, the current efficiency (η) is 82.7% and the electrical energy consumption (W) is 2854 kW·h/t.

The particle size D₅₀ of the copper powder is 81.6µm.

### Example 1.3

The process was carried out in the same manner as described in Example 1.1 expect that the electrolyte solution was kept at a temperature of 30 °C.

The bath voltage is 2.5 V, the current efficiency (η) is 85.1% and the electrical energy consumption (W) is 2476 kW·h/t.

The particle size D₅₀ of the copper powder is 89.2 µm.

### Example 1.4

The process was carried out in the same manner as described in Example 1.1 expect that the electrolyte solution was kept at a temperature of 35 °C.

The bath voltage is 2.6 V, the current efficiency (η) is 87.8% and the electrical energy consumption (W) is 2496 kW·h/t.

The particle size D₅₀ of the copper powder is 100.9µm.

### Example 1.5

The process was carried out in the same manner as described in Example 1.1 expect that the electrolyte solution was kept at a temperature of 45 °C.

The bath voltage is 2.35 V, the current efficiency (η) is 89.16% and the electrical energy consumption (W) is 2222 kW·h/t.

The particle size D₅₀ of the copper powder is 78.4µm.

### Example 1.6

The process was carried out in the same manner as described in Example 1.1 expect that the electrolyte solution was kept at a temperature of 50 °C.

The bath voltage is 2.2 V, the current efficiency (η) is 91.53% and the electrical energy consumption (W) is 2026 kW·h/t.

The particle size D₅₀ of the copper powder is 46.3 µm.

### Comparative Example 1.1

Copper sulfate pentahydrate was dissolved in an aqueous sulfuric acid solution to obtain a solution containing 12 g/L copper ions and 142 g/L free sulfuric acid as the electrolyte solution. The solution was poured into the electrolytic cell and kept at a temperature of 25 °C. An anode of phosphorus copper plate and a cathode of titanium plate were arranged in the electrolytic cell at a distance of 5 cm. The electrolytic deposition was conducted by applying a direct current with a current density of 13 A/dm² for 15 minutes. Then, the obtained copper particles were removed from the cathode and isolated from the electrolyte solution. The collected copper particles were filtered with vacuum filtration and washed by DI water, dried at a temperature of 60 °C in a vacuum drying oven, and then subjected to a reduction treatment by heating to 500 °C in a reducing atmosphere of hydrogen.

The bath voltage is 2.3V, as determined by *Kocour* power supply, the current efficiency (η) is 79.86% and the electrical energy consumption (W) is 2428 kW·h/t. Thick dendritic crystals were observed via SEM for the copper powder, as shown in Figure 2.

The copper powder has a particle size D₅₀ of 99.3 µm.

### Example 2 Production of Silver powder

### Example 2.1

Black Ag₂O was dissolved in an aqueous diluent solution of methanesulfonic acid (MSA) to provide a solution containing 108 g/L of silver ions and 15.25 g/L of free methanesulfonic acid as the electrolyte solution. The solution was poured into the electrolytic cell and kept at a temperature of 50 °C. An anode of pure silver plate and a cathode of stainless steel plate were arranged in the electrolytic cell at a distance of 3.5 cm. The electrolytic deposition was conducted by applying a direct current with the current density of 5 A/dm² for 15mins. Then, the obtained silver particles were removed from the cathode and isolated from the electrolyte solution. The collected silver particles were filtered with vacuum filtration and washed by DI water, dried at a temperature of 60 °C in a vacuum drying oven.

The bath voltage is 1.23V, as determined by *Kocour* power supply, the current efficiency (η) is 98% and the electrical energy consumption (W) is 312 kW·h/t. Granular crystals were observed via SEM for the silver powder, as shown in Figure 3.

The particle size D₅₀ of the silver powder is 328.8 µm and D₉₀ is 525.4µm.

It was observed that the silver particles were deposited on the cathode with slow and slight dendritic growth, as shown in Figure 4.

### Example 2.2

The process was carried out in the same manner as described in Example 2.1 expect the electrolyte solution was kept at a temperature of 25 °C.

The bath voltage is 1.5 V, the current efficiency (η) is 95% and the electrical energy consumption (W) is 392 kW·h/t.

The particle size D₅₀ of the silver powder is 545.1 µm and D₉₀ is 966.9µm.

### Example 2.3

The process was carried out in the same manner as described in Example 2.1 expect the electrolyte solution was kept at a temperature of 40 °C.

The bath voltage is 1.26 V, the current efficiency (η) is 96% and the electrical energy consumption (W) is 326 kW·h/t.

The particle size D₅₀ of the silver powder is 571.5 µm and D₉₀ is 920.1 µm.

### Comparative Example 2.1

Black Ag₂O was dissolved in an aqueous diluent solution of nitric acid (HNO₃) to provide a solution containing 108 g/L silver ions and 10 g/L free nitric acid as the electrolyte solution. The solution was poured into the electrolytic cell and kept at a temperature of 25 °C. An anode of pure silver plate and a cathode of stainless steel plate were arranged in the electrolytic cell at a distance of 3.5 cm. The electrolytic deposition was conducted by applying a direct current with a current density of 5 A/dm² for 15 minutes. Then, the obtained silver particles were removed from the cathode and isolated from the electrolyte solution. The collected silver particles were filtered with vacuum filtration and washed by DI water, dried at a temperature of 60 °C in a vacuum drying oven.

The bath voltage is 1.4V, the current efficiency (η) is 95.04% and the electrical energy consumption (W) is 366 kW·h/t. Granular crystals were observed via SEM for the silver powder, as shown in Figure 5. The particle size D₅₀ of the silver powder is 78.7 µm and D₉₀ is 758.6 µm.

It was observed that the silver particles were deposited on the cathode with quick and severe dendritic growth, especially at the corner of the cathode, as shown in Figure 6.

### Comparative Example 2.2

The process was carried out in the same manner as described in Comparative Example 2.1 expect the electrolyte solution was kept at a temperature of 40 °C.

The bath voltage is 1.11V, the current efficiency (η) is 96% and the electrical energy consumption (W) is 287 kW·h/t.

The particle size D₅₀ of the silver powder is 395.2 µm and D₉₀ is 648.1 µm.

### Comparative Example 2.3

The process was carried out in the same manner as described in Comparative Example 2.1 expect the electrolyte solution was kept at a temperature of 50 °C.

The bath voltage is 1.04V, the current efficiency (η) is 98% and the electrical energy consumption (W) is 264 kW·h/t.

The particle size D₅₀ of the silver powder is 340.3 µm and D₉₀ is 1167.3 µm.

As shown in Figures 7 and 8, the silver powders produced according to the present invention at a temperature of above 40 °C have particle sizes at least comparable to those of the silver powders produced conventionally with the nitric acid electrolyte system.

## Claims

1. A process for production of a powder of metal in an electrolytic cell comprising an anode made of the metal, a cathode and an electrolyte solution, which comprises
a) anodic dissolution to form ions of the metal in the electrolyte solution and cathodic deposition of metal particles from the electrolyte solution,
b) removal of the metal particles from the cathode into the electrolyte solution, and
c) isolation of the metal particles from the electrolyte solution,
wherein
- the metal is copper or silver, and
- the electrolyte solution comprises (i) an alkane sulfonic acid or alkanol sulfonic acid and (ii) a soluble metal salt of an alkane sulfonic acid or alkanol sulfonic acid.

2. The process according to claim 1, wherein the alkane sulfonic acid is selected from C₁-C₁₂-alkane sulfonic acids, preferably C₁-C₆-alkane sulfonic acids.

3. The process according to claim 1, wherein the alkanol sulfonic acid is selected from C₂-C₁₂-alkanol sulfonic acids, preferably C₂-C₆-alkanol sulfonic acids.

4. The process according to claim 2, wherein the alkane sulfonic acid is selected from methanesulfonic acid, 1-ethanesulfonic acid, 1-propanesulfonic acid, 2-propanesulfonic acid, 1-butanesulfonic acid, 2-butanesulfonic acid, 1-pentanesulfonic acid, 1-hexanesulfonic acid, 1-decanesulfonic acid, 1-dodecanesulfonic acid, methanedisulfonic acid, 1,1-ethanedisulfonic acid, 1,2-ethanedisulfonic acid, 1,1-propanedisulfonic acid, 1,3-propanedisulfonic acid, 1,1-butanedisulfonic acid, 1,4-butenedisulfonic acid, and any combinations thereof.

5. The process according to any of claims 1 to 4, wherein step a) is carried out at a temperature in the range of 20 °C to 70 °C, preferably 30 °C to 60 °C, more preferably 40 to 50 °C.

6. The process according to claim 5, wherein silver powder is produced and step a) is carried out at a temperature in the range of 40 to 50 °C, preferably 45 to 50°C.

7. The process according to claim 5, wherein copper powder is produced and step a) is carried out at a temperature in the range of 40 to 50 °C.

8. The process according to any one of claims 1 to 7, which further comprises a step of anti-oxidation of the metal particles, preferably a step of reduction under an atmosphere of hydrogen.

## Patentansprüche

1. Verfahren zur Herstellung eines Metallpulvers in einer Elektrolysezelle, die eine Anode aus dem Metall, eine Kathode und eine Elektrolytlösung umfasst, das Folgendes umfasst:
a) anodische Auflösung unter Bildung von Ionen des Metalls in der Elektrolytlösung und kathodische Abscheidung von Metallpartikeln aus der Elektrolytlösung,
b) Entfernung der Metallpartikel von der Kathode in die Elektrolytlösung und
c) Isolierung der Metallpartikel aus der Elektrolytlösung,
wobei
- es sich bei dem Metall um Kupfer oder Silber handelt und
- die Elektrolytlösung (i) eine Alkansulfonsäure oder Alkanolsulfonsäure und (ii) ein lösliches Metallsalz einer Alkansulfonsäure oder Alkanolsulfonsäure umfasst.

2. Verfahren nach Anspruch 1, wobei die Alkansulfonsäure aus C₁-C₁₂-Alkansulfonsäuren, vorzugsweise C₁-C₆-Alkansulfonsäuren, ausgewählt wird.

3. Verfahren nach Anspruch 1, wobei die Alkanolsulfonsäure aus C₂-C₁₂-Alkanolsulfonsäuren, vorzugsweise C₂-C₆-Alkanolsulfonsäuren, ausgewählt wird.

4. Verfahren nach Anspruch 2, wobei die Alkansulfonsäure aus Methansulfonsäure, 1-Ethansulfonsäure, 1-Propansulfonsäure, 2-Propansulfonsäure, 1-Butansulfonsäure, 2-Butansulfonsäure, 1-Pentansulfonsäure, 1-Hexansulfonsäure, 1-Decansulfonsäure, 1-Dodecansulfonsäure, Methandisulfonsäure, 1,1-Ethandisulfonsäure, 1,2-Ethandisulfonsäure, 1,1-Propandisulfonsäure, 1,3-Propandisulfonsäure, 1,1-Butandisulfonsäure, 1,4-Butendisulfonsäure und beliebigen Kombinationen davon ausgewählt wird.

5. Verfahren nach einem der Ansprüche 1 bis 4, wobei Schritt a) bei einer Temperatur im Bereich von 20 °C bis 70 °C, vorzugsweise 30 °C bis 60 °C, weiter bevorzugt 40 °C bis 50 °C, durchgeführt wird.

6. Verfahren nach Anspruch 5, wobei Silberpulver hergestellt wird und Schritt a) bei einer Temperatur im Bereich von 40 bis 50 °C, vorzugsweise 45 bis 50 °C, durchgeführt wird.

7. Verfahren nach Anspruch 5, wobei Kupferpulver hergestellt wird und Schritt a) bei einer Temperatur im Bereich von 40 bis 50 °C durchgeführt wird.

8. Verfahren nach einem der Ansprüche 1 bis 7, das ferner einen Schritt der Antioxidation der Metallpartikel umfasst, vorzugsweise einen Schritt der Reduktion unter Wasserstoffatmosphäre.

## Revendications

1. Procédé de production d'une poudre de métal dans une cellule électrolytique comprenant une anode composée du métal, une cathode et une solution électrolytique, qui comprend
a) une dissolution anodique pour former des ions du métal dans la solution électrolytique et un dépôt cathodique de particules métalliques à partir de la solution électrolytique,
b) l'élimination des particules métalliques de la cathode dans la solution électrolytique, et
c) l'isolement des particules métalliques de la solution électrolytique,
dans lequel
- le métal est le cuivre ou l'argent, et
- la solution électrolytique comprend (i) un acide alcanesulfonique ou un acide alcanolsulfonique et (ii) un sel métallique soluble d'un acide alcanesulfonique ou d'un acide alcanolsulfonique.

2. Procédé selon la revendication 1, dans lequel l'acide alcanesulfonique est choisi parmi les acides alcanesulfoniques en C₁-C₁₂, de préférence les acides alcanesulfoniques en C₁-C₆.

3. Procédé selon la revendication 1, dans lequel l'acide alcanolsulfonique est choisi parmi les acides alcanolsulfoniques en C₂-C₁₂, de préférence les acides alcanolsulfoniques en C₂-C₆.

4. Procédé selon la revendication 2, dans lequel l'acide alcanesulfonique est choisi parmi l'acide méthanesulfonique, l'acide 1-éthanesulfonique, l'acide 1-propanesulfonique, l'acide 2-propanesulfonique, l'acide 1-butanesulfonique, l'acide 2-butanesulfonique, l'acide 1-pentanesulfonique, l'acide 1-hexanesulfonique, l'acide 1-décanesulfonique, l'acide 1-dodécanesulfonique, l'acide méthanedisulfonique, l'acide 1,1-éthanedisulfonique, l'acide 1,2-éthanedisulfonique, l'acide 1,1-propanedisulfonique, l'acide 1,3-propanedisulfonique, l'acide 1,1-butanedisulfonique, l'acide 1,4-butènedisulfonique et leurs combinaisons.

5. Procédé selon l'une quelconque des revendications 1 à 4, dans lequel l'étape a) est effectuée à une température dans la plage de 20 °C à 70 °C, de préférence de 30 °C à 60 °C, plus préférablement de 40 à 50 °C.

6. Procédé selon la revendication 5, dans lequel une poudre d'argent est produite et l'étape a) est effectuée à une température dans la plage de 40 à 50 °C, de préférence de 45 à 50 °C.

7. Procédé selon la revendication 5, dans lequel une poudre de cuivre est produite et l'étape a) est effectuée à une température dans la plage de 40 à 50 °C.

8. Procédé selon l'une quelconque des revendications 1 à 7, qui comprend en outre une étape d'anti-oxydation des particules métalliques, de préférence une étape de réduction sous une atmosphère d'hydrogène.
